

## UNITED STATES PATENT OFFICE.

WILLOUGHBY STATHAM SMITH, OF NEWTON POPPLEFORD, AND HENRY JOSEPH GARNETT, OF SEVENOAKS, ENGLAND.

MAGNETIC ALLOY AND ITS APPLICATION IN THE MANUFACTURE OF TELEGRAPHIC AND TELEPHONIC CABLES.

No Drawing. Application filed January 8, 1926, Serial No. 80,101, and in Great Britain November 20, 1925.

This invention relates to alloys of nickel, copper and iron, with the addition of small quantities of other elements, and the manufacture therefrom of wire or tape. Such wires or tapes, when heat treated to give high permeabilities in weak fields, can be used in the manufacture of telegraphic and telephonic cables.

In our former specification No. 1,552,769, 10 alloys of nickel, iron and copper were claimed, which comprised nickel at least 71%, iron about 20%, copper about 5% and a small proportion of manganese with or without a fourth element such as tungsten, 15 chromium, silicon, titanium or molybdenum, with the object of increasing the electrical resistance.

As a result of many experiments, we have 20 discovered that alloys, especially useful for the purpose desired, comprise nickel about 76%, iron about 16%, copper about 5% and a small proportion of manganese, particularly when there is an added element adapted to increase the electrical resistance of the 25 alloy.

*Example 1.*

|                | Per cent. |
|----------------|-----------|
| Nickel-----    | 76.75     |
| Copper-----    | 5.00      |
| Iron-----      | 16.00     |
| Chromium-----  | 2.00      |
| Manganese----- | 0.25      |

This alloy, after forging, rolling and drawing to fine wire, was annealed by heating to 900° C. and air cooled. In this condition it had an initial permeability of 7000 with a specific resistance of 44 microhms per 35 cm.<sup>3</sup>

*Example 2.*

|                | Per cent. |
|----------------|-----------|
| Nickel-----    | 75.35     |
| Copper-----    | 5.10      |
| Iron-----      | 17.20     |
| Chromium-----  | 2.10      |
| Manganese----- | 0.25      |

Almost identical results are obtained from this alloy as from that of Example 1. 45

What we claim is:—

1. An alloy comprising nickel about 76%, iron about 16%, copper about 5% and a small quantity of manganese. 50

2. An alloy comprising nickel of an amount about 76% and not less than 75%, iron about 16% and not more than 18%, copper about 5% and a small quantity of manganese. 55

3. An alloy comprising nickel about 76%, iron about 16%, copper about 5%, a small quantity of manganese, and about 2% of a fifth element adapted to increase the electrical resistance of the alloy. 60

4. An alloy comprising nickel of an amount about 76% and not less than 75%, iron about 16% and not more than 18%, copper about 5%, a small quantity of manganese, and about 2% of a fifth element adapted to increase the electrical resistance of the alloy. 65

5. An alloy comprising nickel about 76%, iron about 16%, copper about 5%, a small quantity of manganese, and about 2% of chromium. 70

6. An alloy comprising nickel of an amount about 76% and not less than 75%, iron about 16% and not more than 18%, copper about 5%, a small quantity of manganese and about 2% chromium. 75

In testimony that we claim the foregoing as our invention we have signed our names 80 this tenth day of December, 1925.

WILLOUGHBY STATHAM SMITH.  
HENRY JOSEPH GARNETT.